

Jan. 13, 1931.

J. S. SMYSER

**1,788,600**

## ABRASIVE ARTICLE AND MANUFACTURE OF SAME

Original Filed Feb. 7, 1924 2 Sheets-Sheet 1



Frances  
James S. Smoyer  
by Roberta Balanta Rushman,  
attij's.

Jan. 13, 1931.

J. S. SMYSER

**1,788,600**

ABRASIVE ARTICLE AND MANUFACTURE OF SAME

Original Filed Feb. 7, 1924 2 Sheets-Sheet 2



Fig. 2

Treasurer;  
James S. Mayser;  
by Palito, Palito & Lushman  
attys.

## UNITED STATES PATENT OFFICE

JAMES S. SMYSER, OF BRIGHTON, MASSACHUSETTS

## ABRASIVE ARTICLE AND MANUFACTURE OF SAME

Application filed February 7, 1924, Serial No. 691,149. Renewed April 14, 1930.

This invention relates to articles of manufacture consisting of a support, and a layer of comminuted material deposited thereon; and more particularly to producing and maintaining the physical union of the material and the support. The invention is especially useful in coating strips or sheets of fabric, paper or the like with abrasive particles as hereinafter described in connection with illustrative embodiment.

Objects of my invention are to provide a simple, and efficient method of producing an abrasive surface on a fabric or other article serving as a base, without materially affecting the flexibility or strength of the article; to provide an electrostatic method of continuously, and progressively producing an abrasive coating on a sheet of fabric, or other article, as it is moved in substantially the direction of its surface; to provide an improved coated fabric or other article; and generally to provide an improved method of and apparatus for producing an abrasive coating on an article.

In one aspect my invention contemplates electrostatically applying an abrasive coating to a fabric, or other article serving as a base, by electrostatically projecting abrasive particles into engagement or binding contact with the article being coated, and then forcing the engaged particles into more intimate engagement with the article.

In another aspect, an abrasive coating is electrostatically applied to an electrically non-conducting article by providing a conducting path extending over the article, applying a coating of binding material to the article, and bombarding the last applied coating by a stream of abrasive particles electrostatically charged oppositely to the conducting path of the article.

In still another aspect, the invention provides a fabric or other article coated with a conducting material having a superposed coating of binder material upon which there is deposited a coating of granular material.

The article, when in sheet form, may be coated by moving the sheet continuously in substantially the direction of its surface; dipping a portion of the sheet into a liquid

bath having comminuted conducting material in suspension, to coat the sheet; drying the liquid from the coating to leave a conducting path over the surface of the sheet; making a sliding contact between the conducting portion of the sheet and one terminal of a source of electromotive force; dipping the sheet in a liquid bath of binding material to leave a coating of the binder on the sheet; equalizing the distribution of the binder coating on the sheet; moving the sheet through a stream of abrasive particles which are electrostatically charged by the source of electromotive force with a sign opposite to that of the conducting path of the sheet; equalizing the distribution of abrasive particles over the surface of the sheet, and forcing the particles into more intimate engagement with the sheet.

Methods and apparatus illustrating a species, of which my invention is a genus, are described more fully hereinafter in connection with the accompanying drawings, in which:

Fig. 1 is an elevation, in section diagrammatically showing apparatus for preparing an abrasive coating on a sheet of fabric;

Fig. 2 is a plan of a portion of Fig. 1;

Fig. 3 is an enlarged view of a portion of Fig. 1;

Figs. 4, 5, 6 and 7 are cross sections of a fabric in successive stages, respectively, of the coating operations.

In Fig. 1 the sheet A of fabric, paper, or similar material, is moved substantially in the direction of its surface and directed by rollers so that it passes continuously through a series of zones B, C, D and E, in each one of which, the sheet is subjected to a different operation.

The sheet A feeds from the roll 10 in the direction indicated by the arrow into the coating zone B where it passes around rollers 11, and dips into the liquid bath 12 in tank 13, the liquid having in suspension granular or comminuted graphite or other conducting material. The liquid is preferably non-corrosive and without appreciable physical or chemical effect upon the sheet when used primarily to suspend the conducting par-

ticles; it may be water or other suitable liquid. The sheet passes between the rollers 14 which remove the excess of the mixture from the sheet, resulting in a substantially uniform distribution of conducting material throughout. The rollers 15 direct the sheet through a drying zone C within the chamber 16, having a heating element 17, such as a steam pipe, or other heater. The liquid upon drying from the coating on the sheet leaves the conducting material distributed over the surface as a conducting path. The brush 18 in contact with the sheet is connected to the positive terminal of the source of electro-motive force 19 which electrifies the conducting path of the sheet with a charge of positive sign.

Rollers 20 direct the sheet through the zone D, in which, a coating of binding material is applied to the sheet as it dips into the liquid bath 21 of binding material, such as paraffin, or other suitable binder, preferably electrically nonconducting, in tank 22, heated by a steam pipe (not shown), or other suitable means. The rollers 24 remove the excess liquid and distribute the coating uniformly over the surface to equalize its thickness.

In the zone E, a coating of abrasive is electrostatically applied to the sheet. The hoppers 30 for containing abrasive particles of emery, carborundum, pumice, or other suitable abrasive material having the size of particle with which it is desired to coat the sheet, discharge through spouts 31 into the cylindrical electrifying chambers 32, preferably of electrically insulating material, disposed on opposite sides of the upwardly moving sheet. The nozzles 33 discharge air into the conduits 34 (see Fig. 3), these conduits having apertures which admit the moving air at suitable pressure to the abrasive container to produce a condition in which the abrasive particles are temporarily suspended in the atmosphere of the container through orifices 38 into the zone of the electrical discharge, which takes place between the needles 37 mounted on bus-bars 36 and the conducting sheet.

Bus bars 36 are connected preferably to the negative terminal of source of electro-motive force 19 by means of leads 39, the effective potential of the source 19 being adjusted to such a value, e. g. 18000 volts, more or less, that the abrasive particles in chamber 32 become electrified with a negative charge, and together with the air admitted through nozzle 33 discharge through slot 38 as a stream of electrified particles which are electrostatically propelled toward the positively charged sheet A, the solid particles bombarding and coming into engagement with the binder coating on the sheet. It will be seen that the electrostatically propelled abrasive particles emerging from each of the ori-

fices 38 become deposited as a thin blanket on the sheet A as it passes through the discharge zone.

The housing 40 for apparatus in the zone E prevents loss of the abrasive particles which fail to become attached to the sheet A, and is preferably constructed of insulating material. Conduit 41 is connected to an exhaust pump (not shown) and exhausts air from the housing 40 in the direction indicated by the arrow, the end of conduit 41 being covered by a screen 42 which sifts the abrasive particles from the air before entering the conduit. Air free from abrasive particles is admitted through openings 43, 44 and 45, thus tending to clarify the air within the housing and together with the air discharged through slots 38 causing a flow of the air and drift of the abrasive particles around the baffle diaphragms 46 as indicated by the arrows, the baffles tending to cause a precipitation of the particles at one end of the housing as indicated by the accumulation 47 which also includes the abrasive sifted by the screen 42. Owing to the reduced air pressure in housing 40 when air is exhausted through conduit 41, air may be fed through nozzles 33 directly from the atmosphere, but if a greater flow is desired compressed air may be fed through these nozzles.

Rollers 48 between which the sheet passes, after being coated with the abrasive, equalizes the distribution of abrasive material on the surface of the sheet and forces the abrasive particles into more intimate engagement with the sheet which then passes upward and is wound on the roll 49. The sheet may be propelled by rotation of the roll 49 or one or more of the rollers with which the sheet contacts between rolls 10 and 49.

Figure 4 shows the appearance of a simple fabric sheet A, of electrically insulating or poorly conducting material, having a warp 50 and a woof 51, before the sheet has entered the coating zone B. Fig. 5 shows the particles 52 of graphite or other conductor distributed over the surface of the fabric after the liquid from the batch 12 has been evaporated from the surface in the drying zone C and before the sheet has entered the coating zone D. Fig. 6 shows the sheet A with the coating 53 of paraffin, or other binding material, before the sheet enters the coating zone E. Fig. 7 shows the completed abrasive sheet having a coating 54 of abrasive particles distributed over the binder coating on each side of the sheet A.

By virtue of the electrostatic charges upon the abrasive particles as they pass to the fabric they are held apart by electrostatic repulsion and consequently are distributed far more effectively than is possible without the use of an electrostatic field. Thus the abrasive material may be deposited in any degree of depth, from an extremely thin deposit ap-

proximately one particle thick to a thick deposit, and in any case the particles are distributed with great uniformity. By coating the fabric upon both sides its usefulness is practically doubled and by virtue of the 5 roughness of the rear side the article can be used more effectively with less danger of slippage in the fingers.

While certain materials have been mentioned in disclosing an example of how the 10 invention may be carried out, it is to be understood that the materials specifically named are not necessary to the invention but may be replaced by other suitable materials. It is obvious that the sheet may be treated 15 in the various zones B, C, D and E by various modifications of the apparatus disclosed within the knowledge of those skilled in the art.

The method, and apparatus disclosed for 20 carrying out the method, permit of producing an abrasive coating on sheet fabric or other articles, particularly those in which it is desired to provide a certain degree of elasticity or flexibility, without objectionally 25 stiffening the sheet or otherwise materially affecting those properties of the sheet which it is desired to preserve.

I claim:

1. Apparatus for applying coatings to 30 electrically non-conducting sheet material, comprising means for feeding the sheet in substantially the direction of its surface, means for coating the moving sheet with a conducting material, means for applying a coating of binder material over said conducting coating, and means for electrostatically 35 bombarding the binder coating with electrically charged particles to produce a coating upon said binder coating.

2. Apparatus for applying coatings to 40 electrically non-conducting sheet material, comprising means for propelling the sheet substantially in the direction of its surface, means for applying to the sheet a coating of liquid having conducting particles in 45 suspension, means for drying the liquid to leave conducting particles as a coating on the sheet, means for applying a coating of binder material to the sheet, and means for electrically 50 projecting a stream of granular matter into engagement with the binder coating to apply a superficial coating to the sheet.

3. The method of electrostatically depositing a coating upon an article comprising 55 agitating granular matter in the presence of an electric field, confining movements of the agitated particles to a restricted zone, and electrostatically projecting the electrified 60 particles outwardly from the restricted zone to the object to be coated.

4. The method of preparing an abrasive 65 coating on fabric or similar material, which comprises continuously moving the sheet in substantially the direction of its surface, pro-

gressively dipping the sheet in a liquid bath having finely divided conducting material in suspension, drying up the liquid left as a coating on the sheet and leaving the suspended particles deposited on the sheet to 70 form a conducting path over the surface of the sheet, coating the sheet with a binder, equalizing the thickness of the binder coating, electrostatically projecting a stream of abrasive particles against the sheet, and forcing the abrasive particles into closer engagement with the sheet.

5. The method of preparing an abrasive coating on a sheet of fabric or similar material, which comprises moving the sheet substantially in the direction of its surface, dipping the sheet in a liquid bath having comminuted conducting material in suspension, drying up the liquid left as a coating on the sheet and leaving the suspended material deposited to 80 form a conducting path over the surface of the sheet, dipping the sheet in a bath of liquid binding material, and electrostatically depositing a coating of abrasive particles on the binder.

6. The method of preparing an abrasive coating on a sheet of fabric or similar material, which comprises passing the sheet through a liquid having comminuted conducting material in suspension, withdrawing the sheet from the liquid and drying the liquid to leave a coating of conducting material on the sheet, coating the sheet with a binding material, and electrostatically projecting abrasive particles into engagement 90 with the coating of binding material.

7. The method of preparing an abrasive coating on a sheet of fabric or similar material, which comprises coating the sheet with an electrically conducting material electrostatically projecting abrasive particles into engagement with the sheet and forcing the engaged abrasive particles into more intimate engagement with the sheet.

8. The method of preparing an abrasive coating on a sheet of fabric or similar material, which comprises continuously moving the sheet in substantially the direction of its surface, progressively coating the sheet with a liquid having comminuted conducting material in suspension, progressively drying the liquid to leave the suspended material as a conductive coating on the sheet, progressively coating the sheet with a binding material, and progressively bombarding the sheet with a stream of abrasive particles electrically charged oppositely to the conducting coating of the sheet.

9. The method of preparing an abrasive coating on a sheet of fabric or similar material, which comprises continuously moving the sheet in substantially the direction of its surface, progressively depositing a conducting coating on the sheet, projecting a stream of abrasive particles electrified oppo-

- sitely to the conducting coating into engagement with the sheet, and securing the engaged abrasive particles into more intimate engagement with the sheet.
- 5 10. The method of preparing an abrasive coating on an electrically non-conducting base, which comprises coating the base with an electrically conducting material, coating the conducting material with a binding material, and electrostatically projecting a stream of abrasive particles into engagement with the binder coating.
- 15 11. The method of making an abrasive article which comprises rendering a sheet of fabric or the like both conductive and adhesive and by oppositely charging the conductive sheet and comminuted abrasive material adjacent thereto, electrostatically depositing a layer of said material upon the adhesive surface thereof.
- 20 12. The method of coating a sheet of material with abrasive particles which comprises rendering the sheet both conductive and adhesive and, by oppositely charging the conductive sheet and abrasive particles in the region of the sheet, electrostatically depositing the abrasive particles upon the adhesive surface of the sheet.
- 25 13. The method of coating a sheet of material with abrasive particles which comprises rendering the sheet both conductive and adhesive, continuously agitating a supply of abrasive particles in an enclosed region, continuously feeding the sheet along a path associated with said region, and by oppositely charging the conductive sheet and abrasive particles in said region electrostatically embedding the particles upon the adhesive surface of the sheet.
- 30 14. Apparatus for applying adhesive material to an electrically conducting surface and depositing thereon finely divided particles under the influence of an electrostatic field, comprising means for moving the surface in substantially the direction of its length, means for applying adhesive material to the surface, and means for electrostatically bombarding the adhesive material with electrically charged particles to produce a coating upon said adhesive material.
- 35 15. Apparatus for applying finely divided particles to a surface previously rendered electrically conducting and adhesive, comprising means for producing an electrostatic field in a region containing finely divided particles and means for moving the surface through said electrostatic field.
- 40 16. The method of electrostatically depositing finely divided material particles upon an article, which comprises establishing an electrostatic field, dispersing the finely divided material particles to form a suspension in a region containing the electrostatic field, confining movements of said particles to a restricted zone and electrostatically projecting them to the article to be coated.
- 45 17. The method of spreading an abrasive coating on a sheet of fabric or similar material which comprises treating the sheet to render it electrically conductive and mechanically adhesive, establishing an electrostatic field of force between the surface to be coated and a charged conductor of opposite polarity to that of the sheet and adjacent thereto, conveying finely divided abrasive particles into the electrostatic field of force and moving the surface progressively and in substantially its own plane through the electrostatic field of force whereby the abrasive particles may, by the action of the electrostatic field of force upon them, be deposited thereon.
- 50 18. The method of spreading a coating of finely divided particles on a sheet of fabric or similar material which comprises treating the sheet to render it electrically conductive and mechanically adhesive, establishing an electrostatic field of force between the surface to be coated and a charged conductor of opposite polarity to that of the sheet and adjacent thereto, conveying the finely divided particles into the electrostatic field of force, and moving the surface progressively and in substantially its own plane through the electrostatic field of force whereby the finely divided particles may, by the action of the electrostatic field of force upon them, be deposited thereon.
- 55 19. Apparatus for depositing finely divided particles on the surface of a fabric or other material comprising means for treating the fabric to render it electrically conductive and mechanically adhesive, means for establishing an electrostatic field of force between two electrodes of opposite polarity one of which is in electrical contact with the surface of the fabric, means for conveying the finely divided particles into the electrostatic field of force where, under its influence, they will be deposited on the surface of the fabric, and means for progressively moving said surface in substantially the direction of its length.
- 60 20. Apparatus for depositing finely divided abrasive particles on the surface of a fabric or other material comprising means for treating the fabric to render it electrically conductive and mechanically adhesive, means for establishing an electrostatic field of force between two electrodes of opposite polarity one of which is in electrical contact with the surface of the fabric, means for conveying the finely divided abrasive particles into the electrostatic field of force where, under its influence, they will be deposited on the surface of the fabric, and means for progressively moving said surface in substantially the direction of its length.
- 65 21. The method of coating, with pulverized material, a surface that is both electrically conductive and mechanically adhesive com-

prising establishing an electrostatic field of force between two electrodes of opposite polarity one of which is in electrical contact with the surface to be coated, conveying the pulverized material into the electrostatic field of force under the action of which it will be translated to the surface to be coated, and subjecting successive parts of the surface to the combined action of the electrostatic field of force and the pulverized material in a manner that will be substantially continuous.

5 22. The method of coating, with finely divided abrasive material, a surface that is both electrically conductive and mechanically adhesive comprising establishing an electrostatic field of force between two electrodes of opposite polarity one of which is in electrical contact with the surface to be coated, 10 conveying the finely divided abrasive material into the electrostatic field of force under the action of which it will be translated to the surface to be coated, and subjecting successive parts of the surface to the combined 15 action of the electrostatic field of force and the finely divided abrasive material in a manner that will be substantially continuous.

20 23. The method of spreading a coating of finely divided material upon an electrically 25 conductive surface, which comprises establishing an electrostatic field of force between two electrodes of opposite polarity, one of which is in electrical contact with the surface to be coated, conveying the finely divided material into the electrostatic field of force under the action of which it will be translated to the surface to be coated, and bonding the 30 finely divided material to the surface to be coated.

35 40 Signed by me at Boston, Massachusetts, this 15th day of January, 1924.

JAMES S. SMYSER.

45

50

55

60

65